

# UNITED STATES PATENT OFFICE.

HENRY W. ADAMS, OF NEW YORK, N. Y.

## IMPROVEMENT IN FACTITIOUS OILS.

Specification forming part of Letters Patent No. 12,614, dated April 3, 1855.

*To all whom it may concern:*

Be it known that I, HENRY W. ADAMS, of the city, county, and State of New York, have invented a new and useful Improvement in the Manufacture and Composition of Lubricating and Burning Oils; and I do hereby declare that the following is a full and exact description thereof.

The nature of my invention consists in mixing crude turpentine with the fixed oils and filtering the said mixtures after neutralizing any acid which may be in the turpentine by an alkali.

To enable others skilled in the art to make and use my invention, I will proceed to describe its composition and manufacture.

To make a good lubricating and burning oil I take seven gallons of lard-oil and one gallon of crude turpentine, as it comes into market from the pine tree, and mix them together. This is done by stirring the mixture a few minutes, when a perfect solution of the crude turpentine takes place. I first neutralize any acid which may be present in the turpentine, if for machinery oil, but not for burning, if any, by lime, soda, potash, ammonia, or any suitable alkali, and subsequently filter the said mixture, whereupon the oil is clear, transparent, and ready for use, either for lubricating or burning in a common lamp without smoke. The benefits of this oil are, that it has a much better body than lard-oil for lubricating, will stand better weather, and is much cheaper. For coarser machinery I have mixed successively

six, five, four, three, two, and one part of lard and other suitable oils with one part of crude turpentine and used these several mixtures with success upon machinery and for burning in lamps. Even one part of lard-oil and two parts of crude turpentine will mix together perfectly and filter clear and answer for very slow and heavy bearings.

By mixing linseed or any other drying oil with crude turpentine as above a good painter's oil is formed, especially for dark-colored paints. By mixing any of the fish-oils with crude turpentine in the same manner as above they are rendered whiter and sweeter, and good tanner's oil is produced. Whale-oil and crude turpentine thus rendered light colored and sweet make a good cordage-oil.

I am aware that animal and vegetable oils have been mixed together and used for lubricating, painting, tanning, and burning purposes. I therefore claim no such mixtures; but crude turpentine is not an oil, and therefore its mixture with fixed oils is a new composition of matter.

What I claim as my invention, and desire to secure by Letters Patent, is—

The use of crude turpentine in a mixture made with it and the fixed oils, in the manner and for the purposes hereinbefore substantially set forth.

HENRY W. ADAMS.

Witnesses:

DANIEL M. HASKELL,  
JAMES R. HASKELL.